

## UNITED STATES PATENT OFFICE

GUSTAV KOMAREK, OF CHICAGO, ILLINOIS, ASSIGNOR TO BERWIND FUEL COMPANY OF DELAWARE, OF CHICAGO, ILLINOIS, A CORPORATION OF DELAWARE

## BRIQUETTE AND PROCESS FOR MAKING THE SAME

No Drawing.

Application filed December 2, 1929. Serial No. 411,209.

The present invention relates to fuel briquettes and has for its object to provide a briquette which will be substantially dust proof and also of improved character for combustion purposes.

This application is a continuation in part of my application Serial No. 372,545, filed June 20, 1929, wherein is set forth a briquette and method of forming same employing a deliquescent material either added to the mixture of carbonaceous material and binder before manufacture in the briquetting machine or the deliquescent material in solution or dry form is applied to the surface of the prepared briquette, in each case so that it would be free to exert its active hygroscopic properties.

This invention contemplates the application to the surface of the briquette of a solution of a deliquescent material, also means for causing the material to adhere, and means for protecting the surface of the briquette against abrasion and dusting.

With certain types of briquette material it is not practical to add the deliquescent material to the mass before the briquette is shaped and in other cases it is not always possible to effectively apply the deliquescent coating to the surface of the prepared briquette without some additional treatment. These difficulties are usually traceable to the binder employed or to the smooth or greasy nature of the surface of the briquette, making it difficult for a solution to be effectively applied.

Wherever such objections are found, the present invention is applicable, and it comprises the use of heat in impregnating the surface of the briquette with the solution of deliquescent material, the heat being employed by heating the briquette itself, or the solution, or both. The heat will cause the deliquescent material to adhere to the surface for a considerable period of time and exert its hygroscopic action to prevent dusting. In addition to the hygroscopic material I have

also found it desirable in some cases to apply therewith a film forming material which will serve to retain the deliquescent material in the briquette, add strength to the surface of the briquette and additionally minimize dusting due to abrasion. The film forming material will act as a binder and also provide a protective envelope about the briquette.

The deliquescent material which I propose to employ in solution comprises one or more of a series including calcium chloride, magnesium chloride, and potassium carbonate. The film forming material may also be deliquescent in its nature, although not necessarily so, and may consist of sulphite liquor or some other suitable binder capable of drying to form a smooth, firm envelope. By strong and firm is meant a film which is not excessively sticky so that when the briquettes are piled, they do not produce a conglomerate which would interfere with handling them. In other words, the coating obtained is but slightly moist or tacky, and can best be described as substantially dry, i. e., relatively dry as compared with a thick sticky mass of an adhesive and deliquescent material indiscriminately mixed and applied. Such a covering would not be abrasion resistant nor have a firm, strong surface.

It is, moreover, an object of my invention to provide a briquette having its surface impregnated with the above mentioned materials and wherein this impregnation may be materially assisted by the step of applying the heated deliquescent solution or mixture with film forming agent to the briquette, preferably while the latter is also in heated condition.

With this method of procedure employing either the deliquescent solution alone or in combination with the film forming agent, and with or without the use of heat, there results a strong firm surface which will be hygroscopic and prevent or minimize the effects of abrasion on the surface of the briquettes. In

this manner there is overcome the objections to dust formation which occur in the conventional methods of manufacturing and handling of briquettes. The strong firm surface of the briquette of this invention is slightly moist or tacky, but is relatively dry in that the briquettes will not be covered with a heavy sticky coating such as would interfere with their proper handling by forming a conglomerate. Furthermore such a thick sticky covering when allowed to dry would cause the surface portions of briquettes to be broken off or torn off in handling, and hence produce exposed surface areas which would crumble and break down the entire surface of the briquette. The substantially dry strong surface film effectively protects the briquette against the results of abrasion while at the same time permitting the hygroscopic effect to be exerted. By the alternative processes above referred to which utilize heat, the formation of the substantially dry deliquescent abrasion resistant coating is facilitated.

In carrying out this invention the solution may be applied to suitable rolls, such as pressing and forming rolls in contact with which the briquette mass is passed; or the solution may be applied to the walls of the molds of the usual briquetting machine. In fact, any suitable means for impregnation may be employed which will coat thoroughly the surfaces of each briquette.

As stated, a solution of hygroscopic material is employed, and this may comprise substantially any deliquescent salt of a class of which calcium chloride, magnesium chloride, and potassium carbonate are examples.

The solutions may comprise up to 60% of deliquescent salts depending obviously upon the nature of the briquette and its surface to be treated. Where the deliquescent material is used alone in the treating solution, the solution is preferably raised to boiling temperature and applied in such condition to the surface of a briquette.

However, it is not necessary at all times to have the temperature at boiling, since there are circumstances where a lower temperature will be satisfactory.

It will be understood, however, that a high temperature is desirable in order to prevent crystallization of the solution which will take place at atmospheric temperature.

In addition to the hygroscopic material above mentioned, it is often desirable to impart to the briquette a film or coating which will strengthen the surface and minimize the possibility of dusting by providing a clean smooth surface which will be unaffected by abrasion in handling.

For this purpose any suitable film forming material may be utilized but I prefer a hygroscopic substance, as, for example, sulphite liquor. The sulphite liquor is preferably mixed with the deliquescent solution already

referred to and the mixture is applied as above described.

The effect of adding the film forming agent is to assist in retaining the deliquescent agent, increase the strength of the surface of the briquette considerably, and prolong the effectiveness of the protection against creation of dust, by acting as a binder and forming an envelop about the briquette.

Moreover, where a mixture of film forming agent and deliquescent material are employed, the mixture need not be heated to the relatively high temperature required where the deliquescent salts are used alone.

It is proposed, as will be understood, to apply a heated solution comprising a mixture of the deliquescent or hygroscopic materials and the film forming agent so as to thoroughly impregnate the briquette.

I have also found in certain cases that an excellent coating or impregnation is obtained where the briquette is treated while in heated condition. In other words, the steps mentioned above produce a very excellently protected briquette if they are applied to the briquette while the latter is in heated condition either instead of heating the solution, or, as preferred, with both the briquette and solution heated.

The percentages of the solution containing the deliquescent salts and sulphite liquor may vary greatly. For instance, as stated, a solution having a percentage of deliquescent salts up to 60% or more may be used and as the temperature of the solution is maintained at a high point, crystallization of the solution is prevented. To this solution may be added a varying percentage of film forming agent such as sulphite liquor depending on the protection desired against dust and also depending on the nature of the coal.

If, for instance, the briquette surface were such that it would liberate a considerable amount of fine dust, then the deliquescent solution should contain a high percentage of the sulphite liquor to produce a strong protective film against creation of dust.

Two very effective solutions which have been employed comprise calcium chloride, 30%, and sulphite liquor 5%; and calcium chloride 40% and sulphite liquor 10%. It will be understood, however, that the deliquescent salts may be used in any advantageous proportions and the quantity of film forming agent in the mixture may likewise be increased or diminished to suit exact purposes. This will be accomplished, of course, by actual test. It may be stated, however, that in my experiments solutions containing as high as 60% deliquescent salts have been effective and likewise mixtures containing up to 30 or 40% of the film forming agent such as sulphite liquor have likewise been effective.

The briquettes produced in accordance with this invention are dust proof since the deli-

quescent solution will maintain the briquette surface hygroscopic and prevent dust while the sulphite liquor will provide a film of considerable strength, thereby preventing or 5 minimizing abrasion on the surface of the briquettes.

The solution containing the deliquescent salts may vary in specific gravity to meet the varying demands of the trade. The desirability of employing the sulphite liquor in connection with the deliquescent solution resides in its effect in creating a film of great strength which will prolong the effectiveness of the protection against the creation of dust. As 10 stated, the addition of the sulphite liquor to the deliquescent salt solution permits of adhesion of the solution to the briquette surface with the solution at a lower temperature than ordinarily necessary with the deliquescent salt solution alone used.

It will be understood that an impregnation with deliquescent material may be followed in an impregnation of film forming material as separate steps if desired.

25 It will be understood, also, that instead of heating either of said solution or a mixture thereof, they may be applied without heating to a briquette, the surface of which is raised to a temperature as will permit the 30 solutions to thoroughly adhere thereto.

With respect to the manner of preparing the briquette in order to raise its temperature, it may be stated that while various means for supplying and maintaining the 35 briquette at increased temperature are possible, we find that such simple expedients as heating with steam, hot water, or direct heat are desirable. The temperature of the briquette to cause proper adhesion and formation of the film will be determined by test as the briquette materials will necessarily 40 vary in character as will also the solutions.

The method of application, as heretofore set forth, comprises passing the briquettes 45 in contact with rolls carrying the solution and these rolls, of course, may be heated in order to maintain the solution at a proper temperature. Also, the solution may be applied to the molds in which the briquette is formed.

50 By reason of the invention herein set forth, the thickness of the coating may be readily controlled and it is often desirable to provide a relatively thick coating and film where briquettes are not to be used for a considerable period after their manufacture. In such a case, a deliquescent solution of greater specific gravity will be employed in order that protection will remain effective for a fairly long time.

The present invention is effective regardless of the binders employed in manufacturing the briquette, and as set forth in my previous application, it is essential that the 55 deliquescent material be applied in sufficient

quantity to permit the due exertion of its hygroscopic properties.

In addition to the difficulties incident to the use of binders, very often the surfaces of the briquette are oily and will not permit of 70 adhesion of a deliquescent solution unless treated in accordance with the present method.

Moreover, the surface of the briquettes are 75 frequently smooth and shiny and of a greasy-like nature, also making it difficult if not impossible, for any liquid solution containing deliquescent salts to adhere to the briquettes. The present invention overcomes all of these 80 objections in that it allows of a deliquescent material being effectively applied to the surface of a briquette as well as a strong film forming agent which will increase the protective action against formation of dust.

In referring to briquettes herein, it will be understood that they may be formed as usual of finely divided carbonaceous material such as anthracite or bituminous coal, coke fines, or petroleum coke. In fact, the invention is applicable to substantially all types of briquettes which have for their principal ingredient finely divided carbonaceous or combustible material.

In addition to the sulphite liquor, herein referred to as the film forming agent, I have 90 found such materials as molasses and starch equally satisfactory for this purpose.

Briquettes having treated surfaces in accordance with the present invention present 100 many important advantages over the untreated conventional briquette. Thus, briquettes with untreated surfaces will educe odors when fired from an incandescent fuel bed in the furnace before the process of shoveling in or replenishing the fuel supply is completed. This is due to the more volatile hydrocarbons contained in the binding materials distilling at comparatively low temperatures. However, the briquette with the 105 treated surface will not educe such odors until much higher temperatures are reached which permits completion of replenishing the fuel supply and closing the furnace doors without being aware of such odors. The reason for this is found in the moist briquette 110 surfaces which not only retards the distillation of the more volatile hydrocarbons, but also produces gases readily combustible at lower temperatures. In actual firing tests, it

115 was shown that while firing briquettes with untreated surfaces a certain amount of smoke would pass out of the furnace. The briquette with the treated surface would create a flame and burn the smoke at a furnace temperature that was the same on both tests, but at which no flame appeared when briquettes with the untreated surfaces were fired.

I claim:

1. A fuel briquette having a heat united 120 deliquescent abrasion resistant coating.

2. A fuel briquette having a heat united deliquescent abrasion resistant coating, said coating comprising a deliquescent substance and a film producing material forming an abrasion resistant film or envelope about the briquette. 14. The process of preparing a fuel briquette which comprises applying a solution of a deliquescent salt and sulfite liquor to the heated surface of a briquette. 15. The process of treating briquettes which comprises heating the briquette and impregnating the heated surface thereof with a heated solution of a deliquescent salt and sulphite liquor. 70
3. A fuel briquette having a heat united deliquescent abrasion resistant coating, said coating comprising an inorganic deliquescent salt, and a binder forming an abrasion resistant film or envelope about the briquette. 10 75
4. A fuel briquette having an abrasion resistant deliquescent coating united thereto, said coating comprising a deliquescent and 15 film producing material which forms a substantially dry and strong exposed abrasion resistant and deliquescent film or envelope about the briquette. 80
5. A briquette comprising combustible material and a surface coating comprising a deliquescent salt and sulphite liquor. 85
6. A briquette comprising combustible material and a surface coating comprising a deliquescent salt and starch. 90
7. A briquette comprising combustible material and a surface coating comprising a deliquescent salt and molasses. 95
8. The process of preparing a fuel briquette which comprises applying a hygroscopic and abrasion resistant coating to the surface of the briquette in the presence of heat and at such a temperature that an abrasion resistant surface skin or envelope will be formed about the briquette having hygroscopic properties. 100
9. The process of preparing a fuel briquette which comprises heating the briquette surface and applying thereto a coating of a deliquescent material and an abrasion resistant film producing substance. 105
10. The process of preparing a fuel briquette which comprises applying to the briquette surface a heated solution of a deliquescent material and an abrasion resistant film producing substance. 110
11. The process of preparing a fuel briquette which comprises heating the briquette surface and applying thereto a heated solution of a deliquescent material and an abrasion resistant film producing substance. 115
12. The process of forming a fuel briquette having a deliquescent abrasion resistant coating united thereto which comprises separately applying a deliquescent material and an abrasion resistant film forming substance to the surface of the briquette to form a strong film or envelope about the briquette without substantially reducing the deliquescence of the coating. 120
13. The process of preparing a fuel briquette having a deliquescent abrasion resistant coating united thereto which comprises applying a heated solution of a deliquescent salt and sulfite liquor to the surface of a briquette. 125
- 100

In testimony whereof I have hereunto set my hand. 75

GUSTAV KOMARLK. 80